

1

2,859,143

## FERRITIC ALUMINUM-IRON BASE ALLOYS AND METHOD OF PRODUCING SAME

Joseph F. Nachman and William J. Buehler, Silver Spring, Md., assignors of one-fourth to Edward A. Gaugler, Butler, Pa., and one-fourth to Stephen Girard Lax, Washington, D. C.

No Drawing. Application August 6, 1954  
Serial No. 448,398

27 Claims. (Cl. 148—2)

(Granted under Title 35, U. S. Code (1952), sec. 266)

The invention described herein may be manufactured and used by or for the Government of the United States of America for governmental purposes without the payment of any royalties thereon or therefor.

The present invention relates to a series of alloys for high temperature and magnetic uses, and more particularly to the method and processing technique essential to produce physically sound high quality materials.

Heretofore, certain known alloys of aluminum and iron possessed excellent oxidation resistance when heated to a high temperature in air. However, such alloys were weak in structure and lacked high temperature strength, and desired malleable characteristics such that they could be formed into any desired shape. To take advantage of the high temperature oxidation and high temperature strength possibilities the aluminum content of these alloys must be rather high [minimum of about 10% Al]. Considerable difficulty, however, was encountered in melting, casting, rolling, and processing, even binary Al-Fe alloys, into cold rolled sheet form when the aluminum content exceeded 10%. Moreover, due to the inherent brittle characteristics of the binary Al-Fe alloys with the Al content exceeding 10% no successful method has been devised heretofore to produce a usable and workable sheet material from such alloys, having strengthening additives such, for example, as Mo, V, Ti, Ta, Cb, Cr, W, and B. Nor was it possible heretofore to hot and cold roll such materials containing three or more of the aforesaid metals into physically sound flexible sheets of any desired and workable thickness.

The present invention contemplates the provision of a new series of ferritic high temperature and magnetic alloys containing non-strategic materials, such, for example, as aluminum-iron and/or a small amount of material such, for example, as Mo, V, Ti, Ta, Cb, Cr, W, and B and the novel processing of such alloys into any desired shape. Moreover, in accordance with the new and improved alloys and processing techniques it has been found that the materials produced in accordance with the present invention possess extremely fine oxidation resistance at elevated temperatures and high temperature strengths which are superior to most commer-

2

cial ferritic type high temperature materials currently being used in high temperature applications.

Furthermore, no prior method has been successfully devised for rolling such component alloys containing Al in excess of 10% into physically sound usable material and processing the alloys into various forms, including thin cold rolled sheets.

An object of the present invention is to provide compositions of ferritic alloys having excellent high temperature strength and oxidation resistance.

Another object of the invention is to provide a new and improved method of making aluminum-iron base alloys into usable material having improved high temperature and magnetic properties.

15 Another object of the invention is to provide a new and improved method of processing aluminum-iron base alloys into workable sheet material characterized by high tensile strength and high resistance to corrosion and oxidation.

20 Another object of the invention is to provide a series of aluminum-iron base materials capable of being extruded by standard hot extrusion methods into usable shapes possessing the magnetic and high temperature properties associated with these alloys.

25 Still another object of the invention is to provide a series of materials with a very high electrical resistivity [160 microhm—Cm] coupled with the excellent high temperature properties suitable for use in electrical resistance heating applications.

30 A further object of the invention is to provide a method for producing a series of materials exhibiting good resistance to wet corrosion, at room temperature, when brought in contact with common corrosive mediums.

35 A still further object of the invention is to provide a method for producing a series of magnetic materials possessing excellent magnetic properties coupled with a high hardness and wear resistance.

40 A still further object of the invention is to provide a series of alloys in usable form such, for example, as sheets, castings and the like, exhibiting second phase precipitation phenomena to strengthen the materials both at room temperature and at elevated temperatures.

45 Other objects and many of the attendant advantages of this invention will be readily appreciated as the same becomes better understood by reference to the following detailed description.

In accordance with the present invention the alloy compositions may consist of 10 to 18% Al, 0 to 5% of any one or any combination of the following elements 50 Mo, V, Cr, Ti, Ta, Cb, W, and B, the remainder of basic alloy being Fe.

Using the methods of fabrication and composition limits in accordance with the present invention the following stress-rupture results were actually achieved, the 55 results being set forth on the following chart or table with the alloy compositions given and the respective heat treatments and material form included.

## High temperature stress-rupture data

| Sample No. | Alloy Composition                       | Form of Alloy Material          | Heat Treatment                                | Stress-Rupture Times in Hrs. Using 25,000 p. s. i. load and tested at 1,200° F. |
|------------|-----------------------------------------|---------------------------------|-----------------------------------------------|---------------------------------------------------------------------------------|
| 1.         | 15.6% Al, Remainder Fe.                 | 0.020" thick cold rolled sheet. | None.                                         | 0.5                                                                             |
| 2.         | 15% Al, 3.3% Mo, Remainder Fe.          | do                              | 1,050° C. for 2 hrs. followed by an air cool. | 47.6                                                                            |
| 3.         | 17.2% Al, 3.3% Mo, Remainder Fe.        | do                              | do                                            | 69                                                                              |
| 4.         | 17.2% Al, 3.3% Mo, Remainder Fe.        | do                              | 900° C. for 2 hrs. followed by an air cool.   | 24                                                                              |
| 5.         | 10% Al, 3.3% Mo, Remainder Fe.          | do                              | 1,050° C. for 2 hrs. followed by an air cool. | 0.25                                                                            |
| 6.         | 13.8% Al, 4% Mo, Remainder Fe.          | do                              | do                                            | 54.4                                                                            |
| 7.         | 18% Al, 3.3% Mo, 0.05% C, Remainder Fe. | do                              | do                                            | 19.3                                                                            |
| 8.         | 14% Al, 2% Mo, 0.3% V.                  | do                              | do                                            | 17.2                                                                            |
| 9.         | 15% Al, 5% Mo, Remainder Fe.            | do                              | do                                            | 61                                                                              |
| 10.        | 16% Al, 1.68% Mo, 0.3% Ti, Bal. Fe.     | do                              | do                                            | 73.2                                                                            |
| 11.        | 16% Al, 1% Ti, Bal. Fe.                 | do                              | do                                            | 9.9                                                                             |

From the foregoing table of stress-rupture data the following conclusions are obvious:

(1) The basic binary alloy containing about 16% Al, the remainder iron, in the cold rolled sheet form, with no heat treatment has a very low high temperature strength.

(2) The addition of elements such as Mo, V, and Ti definitely improve the high temperature strength.

(3) Coupled with the aforesaid additives, maximum high temperature strengths are attained by a heat treatment of about 1050° C. for about 2 hours followed by a still air cool. The effectiveness of this heat treatment can be seen by comparing samples 3 and 4 in the table.

(4) The percentage of aluminum and iron present in the alloy as shown in the table, in combination with the other elements greatly improves the high temperature strength. This can be shown by comparing samples 2 and 5 in the table.

(5) Higher percentages of elements, such as Mo, increase the high temperature strength. However, there is a practical limit on cold rolled sheet material—that limit being the composition where difficulties in cold rolling are encountered.

(6) The addition of the elements such as Mo, V, and Ti is for the purpose of increasing the high temperature strength of the basic Al-Fe alloys by either strengthening the existing ferritic solid solution or by precipitating a strengthening second phase. These element additions appear to have very little effect upon the grain size or oxidation resistance of the resultant alloys.

These sample data given in the table further illustrate the nature of this invention; however, it should be understood that the invention is not restricted to these specific examples.

The high temperature and magnetic alloy of the instant invention may be made, for example, by melting together an alloy of 10 to 18% aluminum, up to 5% strengthening element additives, the remainder of the alloy being iron, forming a casting or shape, solution heat treating the casting to a temperature within the single phase solid solution region. When this has been done the shape or casting is rapidly cooled to a temperature within the multi-phase region, and the casting or shape is maintained at this reduced temperature until at least one other phase has been precipitated. The term "strengthening element" as employed herein and in the appended claims, is defined as an element such, for example, as Mo, V, Ti, Cr, Ta, Cb, W, Ni, and B, or any combination thereof.

## Magnetic data

|    |                           |                                                                                               |
|----|---------------------------|-----------------------------------------------------------------------------------------------|
| 30 | Nominal alloy composition | 16% Al, 3.3% Mo, remainder Fe.                                                                |
|    | Heat treatment            | 1050° C. for one hour, furnace cool to 600° C., hold at 600° C. for 10 minutes, water quench. |
| 35 | $\mu_m$                   | [max. permeability] = 130,000.                                                                |
| 40 | $\mu_{20}$                | [initial permeability] = 6,600.                                                               |
| 45 | $H_o$                     | [coercive force] = 0.017 oersteds.                                                            |
|    | $B_m$                     | [at $H=30$ oersteds] = 5800 gauss.                                                            |

Based upon actual tests and data obtained on these unique alloys fabricated in accordance with the teaching of the present invention, there are certain combinations and quantities of metallic elements that must be alloyed to produce high temperature materials with suitable strength and oxidation resistance. These quantities may be summarized as follows: The aluminum content should be from about 10 to 18% of total alloy by weight. Added to the Al is another type element or elements, such as Mo, V, Ti, Ta, Cb, Cr, B, and W, which are present in the alloy either as a single element added to the Al and Fe, or in combinations of two or more of these elements. The amount of any one or more but not all of the elements Mo, V, Ti, Ta, Cb, Cr, W, and B, present in the alloy may vary from 0% to 5%. When used in combination the proportions of each of the aforesaid elements may be as high as 5%, the remainder of the overall alloy being iron. The three or more components of the alloys however, are composed of basically iron and aluminum with one or more of the elements Mo, V, Ti, Cb, W, and B present.

In addition to the optimum alloy compositions, and alloy fabrication methods to obtain the maximum high temperature stress-rupture strength in these materials it is essential to perform certain heat treating operations upon the fabricated material as hereinbefore set forth in greater detail. By actual tests, the most satisfactory heat treatment consists of heating the alloy to a temperature of about 1050° C. for about two hours followed by a still air cool. This heat treatment cycle was applied to 0.020" thick sheet material, however, if thicker sec-

tions or sheets are heat treated, longer times of holding at 1050° C. and more rapid cooling means may be needed to effect the same heat treating cycle.

Moreover, when a fine grained sheet material is desired the cold rolled sheet alloys may be recrystallized at about 750° C. for 1 hour. By actual tests it has been found that this recrystallized fine grain size is only possible from cold worked sheet alloys.

#### Material fabrication method

The following describes the methods employed for making the three (or more) component aluminum-iron base alloys for high temperature and magnetic applications. These methods have been proven satisfactory as the result of extensive laboratory experience with these alloys, and for this reason should be adhered to in order to produce high ingot yields of good quality and of physically sound material.

#### Melting and casting

The melting of the aforesaid alloys may be performed in any suitable type of melting furnace, such for example, as a vacuum or controlled atmosphere induction furnace. For the purpose of clarity in describing the operations, an example melt of 16% Al, 3.3% Mo, 80.7% Fe will be described. The first step in the melting operation is to melt the iron and molybdenum under vacuum. The melting is preferably carried out in a magnesium oxide crucible. After the elements are completely melted, wet and dry hydrogen gas is passed over the melt. This operation is performed for the purpose of decarburizing and deoxidizing the iron-molybdenum molten solution. Helium is now introduced into the tank to displace the hydrogen. When the gaseous mixture in the furnace chamber no longer supports a combustion, it will be understood that such action removes most all of the hydrogen that may have been dissolved in the molten alloy. Helium is introduced again into the furnace chamber until one atmosphere of helium is present. At this time the 16% of aluminum is added to the melt and the furnace chamber is again evacuated [using a vacuum pump] to a pressure of 5 millimeters of helium. When this pressure is attained, and the optimum pouring temperature reached, the melt is poured. Pouring may be either into a suitable mold for shaping the material into a final cast shape or it may be poured into an ingot or slab-type mold, forming an ingot or slab for subsequent rolling, swaging or extrusion into strips, sheets, rods, wire or other shapes.

The operation of pumping down to 5 millimeters of helium pressure after the aluminum addition and prior to pouring is an important and essential step in the process. First, it removes the hydrogen from the molten alloy, thus producing sound castings. Secondly, coupled with the mold design it promotes a more desirable solidification rate for the molten alloy thus producing a highly desirable fine and equiaxed cast grain size. If the same melt is poured at one atmosphere of helium, using the same mold, a large grained columnar cast structure would result. When the same melt is poured at one atmosphere of helium into a ceramic mold an equiaxed structure results and a much larger grain size is evident. Thus by the aforesaid treatments it is apparent that it is possible to produce the type of cast grain formation and size of cast grain by varying the rate of solidification of the alloy.

By actual test it has been found that casting such alloys in a steel slab mold under a vacuum of 5 mm. of helium and containing 16% Al, 3.3% Mo, and 80.7% Fe produced a desirable fine equiaxed cast grain structure, the casting in a steel slab mold under one atmosphere of helium produced a less desirable large columnar cast grain structure and the casting in a ceramic mold under one atmosphere of helium produced a large and equiaxed cast grain structure.

It will be understood that the formation of a fine equi-

axed cast grain structure is an important step in the production of good quality material. Large columnar cast grain structure causes hot tearing or cracking during fabrication. Hot tearing or cracking is practically nonexistent in slabs with a fine equiaxed cast grain structure.

#### Conditioning cast slabs

Immediately following the pouring, the cast slab should be stripped from the mold while still red hot. The hot slab is then placed in a furnace at 1050° C. for about two hours and allowed to cool with the furnace, about 30° C. drop in temperature per hour. This operation prevents the cast slab from cracking during rapid cooling following solidification after the heat treatment, if desired, the slab may be machined free of surface imperfections before beginning the hot rolling operations. Machined slabs yield a very clean continuous surface after the material subsequently has been hot and cold rolled. Machining the slab as cast without the heat treatment at 1050° C. followed by a furnace cool, will cause the slab to crack severely during hot working.

#### Hot rolling

After melting, casting and conditioning the slab, the hot rolling operation is in order. The slab is hot rolled to about 0.250" in thickness at a temperature of 1050° C. The reductions in thickness between reheatings and the reductions per pass through the mill are based upon the mill capacity and the rate at which the strip loses heat. Rolling is stopped and reheating is necessary when the strip drops in temperature to a dull red heat. At a thickness of about 0.250", the hot rolling is performed at about 950° C. When the strip has been finished to about 0.125" or preferably 0.1", the cold rolling operation is in order.

It has been found during the rolling operation that some of the aforesaid materials can be successfully hot rolled in the Sendzimir Hot Mill reducing a 1.0" slab to about 0.1" thick in one pass.

#### Conditioning prior to cold rolling

Any surface imperfections present on the hot rolled strip may be removed prior to the beginning of the cold rolling operation in the aforesaid manner. The removal of the imperfections will not effect the material. In reality this operation improves the surface of the material for the final cold rolling operation.

#### Cold rolling

This rolling operation is performed at about 575° C., and may be considered cold rolling for the reasons that the temperature is below the recrystallization temperature.

It will be understood that cold rolling denotes cold working the alloy at a temperature below the recrystallization temperature, whereas hot rolling denotes hot working the alloy at a temperature above the recrystallization temperature. In the hot rolling process, for example, the metal is recrystallized during rolling and in the cold rolling process, the crystal structure remains unrecrystallized and the crystals are elongated. Rolling at about 575° C. gives the material a regular cold worked appearance and elongates the grains into long fibered structure. The greater the percentage of cold work, the higher the mechanical properties of the alloy [tensile strength, yield strength, hardness, impact strength, etc.]. Cold rolling may be performed to reduce the material to a relatively thin gage, such, for example, as 0.002 of an inch or thinner.

#### Removal of oxide coating

After rolling the material into strip form of a suitable thickness, it has a naturally formed coating of aluminum and iron oxides upon the surface. If it is desired to remove this coating for any purpose [spot welding,

soldering, brazing, etc.] it may be removed by the following treatment:

Immerse strip in boiling NaOH [20% solution by weight] for a few minutes. Wash in water at room temperature. Immerse strip at room temperature in HNO<sub>3</sub> [30% solution by volume] for a few minutes. Wash in water and thereafter dry.

This cleaning operation does not attack anything but the oxide coating on the surface.

*Forming and shearing of cold worked material*

Cold rolled strip of a reasonable thickness may be formed and sheared if warmed. The exact temperature of warming is dependent upon the forming configuration and material thickness of the alloy.

The slabs or sheets produced by the aforesaid method may be of any desired length and width and characterized by high tensile strength and high resistance to corrosion and oxidation at elevated temperatures. This material is sufficiently ductile to be readily worked or formed into any desired shape without damage or breakage thereof. Furthermore, it has been found by actual test that the metallic sheets produced in accordance with the present invention are about 20% lighter than stainless steel alloys and the physical and chemical characteristics thereof include high tensile strength and high resistance to corrosion and oxidation. Moreover, creep-rupture tests have proven that the aforesaid material is far superior to some forms of the critical stainless steel alloys now being widely used. It has been further found that because of the high electrical resistivity of the aforesaid material, the material is admirably suited for use in heater elements, low temperature furnaces, and other numerous electrical appliances. It has also been found that due to the electrical resistivity and excellent magnetic characteristics of these cold rolled alloys, these alloys are well suited for magnetic applications.

From the foregoing, it will be apparent that new and improved ferritic materials and the method of making same has been invented, wherein such materials are characterized by high tensile strength and high resistance to corrosion and oxidation at elevated temperatures, high electrical resistivity, and which is sufficiently tough and ductile to be readily formed into various forms including thin tape-like strips or sheets and which is well adapted to extrusion.

Obviously many modifications and variations of the present invention are possible in the light of the above teachings. It is therefore to be understood that within the scope of the appended claims the invention may be practiced otherwise than as specifically described.

What is claimed as new and desired to be secured by Letters Patent of the United States is:

1. The method of making a high temperature and magnetic alloy containing from 10 to 18% aluminum, up to 5% of a strengthening element and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250 of an inch thick at a temperature of about 1050° C. followed by hot working the sheet at a temperature of 950° C. from a thickness of 0.250 of an inch thick to a thickness of substantially 0.125 of an inch, and thereafter cold working the sheet to a predetermined thickness at a temperature of 575° C.

2. The method of making a high temperature and magnetic alloy containing from 10 to 18% aluminum and up to 5% of strengthening elements and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick at a temperature of about 1050° C. followed by hot working the sheet at a temperature of 950° C. from a thickness of 0.250 of an inch thick to a thickness of substantially 0.125 of an inch, and thereafter cold working the sheet to the desired thickness at a temperature of about 575° C.

3. The method of making a high temperature and magnetic sheet alloy containing essentially 16% aluminum and up to 5% molybdenum and remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into sheet substantially 0.250" thick at a temperature of about 1050° C. followed by hot working the sheet at a temperature of 950° C. from a thickness of 0.250 of an inch thick to a thickness of substantially 0.125 of an inch, and thereafter cold working the sheet to a desired thickness at a temperature of about 575° C.

4. The method of making a high temperature and magnetic sheet alloy containing essentially 16% aluminum, 3.3% molybdenum, and remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick at a temperature of about 1050° C. followed by hot working the sheet at a temperature of 950° C. from a thickness of 0.250 of an inch thick to a thickness of substantially 0.125 of an inch, and thereafter cold working the sheet to a desired thickness at a temperature of about 575° C.

5. The method of making a high temperature and magnetic sheet alloy containing essentially 16% aluminum, essentially 2% Mo, essentially 0.3% Ti, and the remainder iron, which consists of melting the constituents together to form a molten alloy, forming the molten alloy into an ingot, controlling the solidification rate of the molten alloy to produce an ingot having a fine equiaxed cast grain structure, uniformly heating the ingot while the ingot is still red hot to a temperature of 1050° C., slow cooling the ingot at a rate of about 30° C. per hour until the ingot is substantially at room temperature, machine working the ingot free of surface imperfections,

hot working the ingot above the recrystallization temperature into a sheet substantially 0.125" thick, and cold working the sheet below the recrystallization temperature to a desired thickness.

6. The method of making a high temperature and magnetic sheet alloy containing essentially 16% aluminum, essentially 2% Mo, essentially 0.3% Ti, and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick at a temperature of about 1050° C. followed by hot working the sheet at a temperature of 950° C. from a thickness of 0.250 of an inch thick to a thickness of substantially 0.125 of an inch, and thereafter cold working the sheet to a desired thickness at a temperature of about 575° C.

7. The method of making a high temperature and magnetic sheet alloy containing essentially 16% aluminum, essentially 2% Mo, essentially 0.3% Ti, and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, cooling the ingot slowly to substantially room temperature, removing surface imperfections from the ingot, hot working the ingot above the recrystallization temperature to a sheet of predetermined thickness, and thereafter cold working the sheet below the recrystallization temperature to a reduced thickness.

8. The method of making a high temperature and magnetic sheet alloy containing essentially 16% aluminum, essentially 2% molybdenum, essentially 0.3% vanadium, and the remainder iron, which consists of melting the constituents together to form a molten alloy, forming the molten alloy into an ingot, controlling the solidification rate of the molten alloy to produce an ingot having a fine equiaxed cast grain structure, uniformly heating the ingot while the ingot is still red hot to a temperature of 1050° C., slow cooling the ingot at a rate of about 30° C. per hour until the ingot is substantially at room temperature, machine working the ingot free of surface imperfections, hot working the ingot above the recrystallization temperature into a sheet substantially 0.125" thick, and cold working the sheet below the recrystallization temperature to the desired thickness.

9. The method of making a high temperature and magnetic sheet alloy containing essentially 16% aluminum, essentially 2% molybdenum, essentially 0.3% vanadium, and the remainder iron which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick at a temperature of

10 about 1050° C. followed by hot working the sheet at a temperature of 950° C. from a thickness of 0.250 of an inch thick to a thickness of substantially 0.125 of an inch, and thereafter cold working the sheet to a desired thickness at a temperature of about 575° C.

10. The method of making a high temperature and magnetic sheet alloy containing essentially 16% aluminum, essentially 2% molybdenum, essentially 0.3% vanadium, and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, cooling the ingot slowly to substantially room temperature, removing surface imperfections from the ingot, hot working the ingot above the recrystallization temperature to a predetermined thickness, and thereafter cold working the sheet below the recrystallization temperature to a reduced thickness.

11. The method of making a high temperature and magnetic sheet alloy containing essentially 17½% aluminum, essentially 3.3% molybdenum, and the remainder iron, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick at a temperature of about 1050° C. followed by hot working the sheet at a temperature of 950° C. from a thickness of 0.250 of an inch thick to a thickness of substantially 0.125 of an inch, and thereafter cold working the sheet to the desired thickness at a temperature of about 575° C.

12. The method of making a high temperature and magnetic sheet alloy containing essentially 16% aluminum, essentially 1% titanium, and the remainder iron, for solid solution strength at high elevated temperatures, which consists of melting the constituents together to form a molten alloy, forming the molten alloy into an ingot, controlling the solidification rate of the molten alloy to produce an ingot having a fine equiaxed cast grain structure, uniformly heating the ingot while the ingot is still red hot to a temperature of 1050° C., slow cooling the ingot at about 30° C. per hour until the ingot is substantially at room temperature, machine working the ingot free of surface imperfections, hot working the ingot above the recrystallization temperature into a sheet substantially 0.125" thick, and cold working the sheet below the recrystallization temperature to a desired thickness.

13. The method of making a high temperature and magnetic sheet alloy containing essentially 16% aluminum, essentially 1% titanium, and the remainder iron for solid solution strength at high elevated temperatures, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, slow cooling the ingot at a rate of about 30° C. per hour until the ingot is substantially at room temperature, removing surface imperfections from the ingot, hot working the ingot into a sheet substantially 0.250" thick

at a temperature of about 1050° C. followed by hot working the sheet at a temperature of 950° C. from a thickness of 0.250 of an inch thick to a thickness of substantially 0.125 of an inch, and thereafter cold working the sheet to a desired thickness at a temperature of about 575° C.

14. The method of making a high temperature and magnetic sheet alloy containing essentially 16% aluminum, essentially 1% titanium, and the remainder iron for solid solution strengthening at high elevated temperatures, which consists of melting the constituents in a suitable melting apparatus to form a molten alloy, forming the molten alloy into an ingot, controlling the solidification rate of the molten alloy to produce an ingot having a fine equiaxed cast grain structure, transferring the ingot from the melting apparatus while red hot to a heating apparatus and heat treating the ingot at a temperature of about 1050° C. for a time sufficient to uniformly heat the ingot, cooling the ingot slowly to substantially room temperature, removing surface imperfections from the ingot, hot working the ingot above the recrystallization temperature to a sheet of predetermined thickness, and thereafter cold working the sheet below the recrystallization temperature to a reduced thickness.

15. The method of making a ferritic high temperature and magnetic alloy containing from 10 to 18% aluminum, up to 5% of a strengthening element and the remainder iron, which consists of melting and refining the iron in a magnesium oxide crucible using a vacuum or controlled atmosphere, charging the melt with said element and aluminum, allowing sufficient time to cause thorough mixing, pouring the melt into a mold and allowing it to solidify under helium or suitable inert atmosphere at a pressure of 5 mm. into a slab substantially one inch thick, stripping the slab from said mold while the slab is substantially red hot, heat treating the slab at 1050° C. for about two hours, cooling slab to about room temperature at a rate of substantially 30° C. per hour, machine working the slab to remove surface imperfections, hot working the slab into a sheet substantially 0.250" thick at a temperature of about 1050° C. followed by hot working the sheet at about 950° C. to a thickness of 0.125", and thereafter cold working the sheet to a desired thickness at about 575° C.

16. The method of making a high temperature aluminum-iron base alloy containing 10 to 18% aluminum and up to 5% of a strengthening element and the remainder iron, which consists of melting the constituents together to form a molten alloy, forming the molten alloy into an ingot, controlling the solidification rate of the molten alloy to produce an ingot having a fine equiaxed grain structure, uniformly heating the ingot to a temperature of 1050° C., slow cooling the ingot at a rate of about 30° C. per hour until the ingot is substantially at room temperature, removing surface imperfections from the ingot, hot working the ingot into a sheet of predetermined thickness at a temperature of about 950° C., cold working the sheet at a temperature of about 575° C. to a reduced thickness, immersing the cold worked sheet into a hot agitated 20% solution of NaOH by weight, washing the sheet in water, immersing the sheet in an agitated 30% HNO<sub>3</sub> solution by volume at room temperature, and thereafter washing the sheet in clear water to remove all traces of the HNO<sub>3</sub> and the oxide coating formed during rolling.

17. The method of making high temperature and magnetic aluminum-iron base alloys containing 10 to 18% aluminum, 3.3% molybdenum and the balance essentially iron into sheet material, which consists of melting the constituents in a melting apparatus to form an alloy melt, forming the melt into a slab substantially 1 inch thick in a ceramic mold, stripping the slab from the mold while the slab is red hot, heat treating the slab at a temperature of 1050° C. for about 2 hours, slow cooling the slab to substantially room temperature at a rate of 30° C. per hour, removing surface imperfection 75

from the slab, hot reducing the slab at a temperature of 1050° C. into sheet material substantially 0.250 of an inch thick, hot reducing the sheet material to a thickness of substantially 0.125 of an inch thick at a temperature of 950° C., and thereafter cold reducing the sheet at a temperature of about 575° C. to a desired thickness.

18. The method of making a high temperature and magnetic alloy containing from 10 to 18% aluminum, up to 5% of a strengthening element and the remainder iron, which consists of melting the constituents together and forming the melt into a suitable ingot, and thereafter extruding the ingot at a temperature substantially above the recrystallization temperature, using a suitable pressure and die lubricant, said alloy being subjected to a heat treatment at 1050° C. followed by cooling at a rate sufficient to disorder the atomic structure.

19. The method of making a high temperature and magnetic multi-phase alloy which comprises producing a melt consisting essentially of 10 to 18% aluminum, up to 5% of a strengthening element, and the remainder iron, casting said melt and solidifying the same to produce a fine-equiaxed cast grain structure, solution heat treating said casting to a temperature within the single phase solid solution region, rapidly cooling the casting to a temperature within the multi-phase region, and maintaining the casting at said last named temperature for a period of time sufficient to precipitate at least one other phase.

20. The method of making a high temperature and magnetic multi-phase alloy which comprises producing a melt consisting essentially of 10 to 18% aluminum, up to 5% of a strengthening element, and the remainder iron, casting said melt and solidifying the same to produce a fine-equiaxed cast grain structure, hot working the casting above the recrystallization temperature to a desired shape, solution heat treating said shape to a temperature within the single phase solid solution region, rapidly cooling the shape to a temperature within the multi-phase region, and maintaining the shape at said last named temperature for a period of time sufficient to precipitate at least one other phase.

21. The method of making a high temperature and magnetic multi-phase alloy which comprises producing a melt consisting essentially of 10 to 18% aluminum, up to 5% of strengthening elements including molybdenum and titanium, and the remainder iron, casting said melt and solidifying the same to produce a fine-equiaxed cast grain structure, solution heat treating said casting to a temperature within the single phase solid solution region, rapidly cooling the casting to a temperature within the multi-phase region, and maintaining the casting at said last named temperature for a period sufficient to precipitate at least one other phase.

22. The method of claim 21 wherein the strengthening elements include 3.3% molybdenum and 0.3% titanium.

23. A high temperature and magnetic ferritic alloy consisting essentially of 10 to 18% aluminum, up to 5% strengthening element, and the remainder essentially iron, said alloy being characterized by a recrystallized fine grain size with disordered atomic structure.

24. A high temperature and magnetic ferritic alloy consisting essentially of 10 to 18% aluminum, up to 5% molybdenum, and the remainder essentially iron, said alloy being characterized by a recrystallized fine grain size with disordered atomic structure.

25. A high temperature and magnetic ferritic alloy consisting essentially of 10 to 18% aluminum, up to 5% titanium, and the remainder essentially iron, said alloy being characterized by a recrystallized fine grain size with disordered atomic structure.

26. The method of making a high temperature and magnetic alloy containing from 10 to 18% aluminum, up to 5% of strengthening element, and the remainder essentially iron, which consists of melting the constituents together in a suitable melting apparatus to form a molten

alloy, forming the molten alloy into an ingot, controlling the solidification rate of the molten alloy to produce a fine equiaxed cast grain structure, annealing the solidified ingot at a temperature of about 1050° C. to eliminate stresses therein, cooling the ingot slowly to substantially room temperature to prevent occurrence of further stresses therein, hot working the ingot above the recrystallization temperature to a sheet of predetermined thickness, and thereafter cold working the sheet below the recrystallization temperature to a desired thickness.

27. A method for making a high temperature magnetic ferritic casting which comprises producing a melt consisting essentially of 10 to 18% aluminum, up to 5% of strengthening element, and the remainder essentially iron, casting said melt and controllably solidifying the same to produce a fine equiaxed cast grain structure, annealing said casting at a temperature of about 1050° C. to eliminate stresses therein, and thereafter slowly cooling the

casting while avoiding the occurrence of further stresses therein.

References Cited in the file of this patent

UNITED STATES PATENTS

|    |           |            |                |
|----|-----------|------------|----------------|
| 5  | 1,915,158 | Fahrenwald | June 20, 1933  |
|    | 1,972,248 | Smith      | Sept. 4, 1934  |
|    | 2,230,531 | Digby      | Feb. 4, 1941   |
|    | 2,339,842 | Digby      | Jan. 25, 1944  |
| 10 | 2,523,917 | Payson     | Sept. 26, 1950 |
|    | 2,624,669 | Crafts     | Jan. 6, 1953   |

FOREIGN PATENTS

|    |         |               |               |
|----|---------|---------------|---------------|
| 15 | 370,012 | Great Britain | Apr. 1, 1932  |
|    | 409,355 | Great Britain | Apr. 30, 1954 |

OTHER REFERENCES

Metal Progress, vol. 35, No. 6 (1939), G. J. Comstock, page 576.